

## UNITED STATES PATENT OFFICE.

HARRY DODGE, OF DANVERS, MASSACHUSETTS.

## PROCESS OF TREATING HIDES OR SKINS.

No Drawing.

Application filed May 14, 1927. Serial No. 191,556.

This invention relates to a process of preparing puered skins or hides and has for its object for not only refining the grain of, but also for making the hide or skin uniform to such an extent whereby after the tanning thereof, the quality of the leather produced will be greatly enhanced and under such conditions increasing its value.

A further object of the invention resides in the preparing of puered skins and hides to preserve them for shipment.

A further object of the invention resides in the preparing of puered skins in a wet state for shipment.

15 Further objects of the invention are to provide, in a manner as hereinafter set forth, a process of preparing or treating puered skins or hides for the purpose referred to which is simple, expeditious and efficient in its use, 20 conveniently carried out, and comparatively inexpensive to employ.

An embodiment of a process for treating or preparing puered skins or hides for the purpose referred to and in accordance with 25 this invention will be hereinafter set forth, but it is to be understood that changes, variations and modifications thereof can be resorted to which fall within the scope of the claims hereunto appended.

30 In carrying out the process of treating or preparing puered skins or hides, in accordance with this invention, the hides or skins, under a state of agitation, are subjected to a bath of alum, common salt and water for a few minutes, after which there is added to the bath nitre  $\text{KNO}_3$  and formaldehyde. The hides or skins are again agitated until the grain and flesh substance thereof are cured and preserved. Nitric acid or distilled sulphuric acid could be used in place of nitre, but preferably the nitre is employed, as the result is better.

The alum and salt both preserve the skins or hides. The formaldehyde binds or fastens the substance of the hide or skin together, and the nitre acts as a filler and fills in the hide or skin substance.

45 The amount of alum employed is approximately 1 to 10% of the weight of the skins or hides to be treated, the salt approximately 1 to 10%, the nitre one-half to 5% and the formaldehyde one-quarter to 5%. The water of a desired amount. The potassium

nitrate  $\text{KNO}_3$  base produces a more valuable product than has heretofore been obtained. 55

It has been found that after the skins or hides are treated in the manner as stated, the skin or hide substance is of a better quality and more uniform than obtained by known processes, and after the hide or skin is tanned by any tanning methods, such as chrome, alum, gambia, sumac or bark, the quality of the leather produced is materially increased 60 resulting in a greater value therefor.

The subjecting of the hides or skins to the preservatives, binder and filler as heretofore stated, will preserve them for shipment, as well as permitting shipment thereof in a wet state.

What I claim is:—

1. A process of treating puered skins or hides consisting in subjecting the article to be treated, while under a state of agitation, to a bath of alum, salt and water, then adding to the bath formaldehyde and nitre, then 75 agitating the article being treated while subjected to the action of the alum, salt, formaldehyde and nitre.

2. A process of treating puered skins or hides consisting of subjecting the article to be treated, while under a state of agitation, to a bath of alum, salt and water, the proportion of the alum being approximately 1 to 10% of the weight of the article and the proportion of the salt being the same, then 80 adding to the bath formaldehyde and nitre with the proportion of the formaldehyde being one-quarter to 5% of the weight of the article and the proportion of the nitre being one-half of 5% with respect to the weight of 85 the article, then agitating the article while subjected to the action of the alum, salt, nitre and formaldehyde for an appropriate period.

3. In a process of treating or preparing puered hides or skins the subjecting of the latter to a bath consisting of water, alum, salt, formaldehyde and nitre.

4. In a process of treating or preparing hides or skins the subjecting of the latter to a bath consisting of water, alum, salt, formaldehyde and nitre, the proportion of the alum and salt being 1 to 10% with respect to the weight of the article or articles being treated, the proportion of the formaldehyde being one-quarter to 5% with re- 100 105

spect to the article or articles being treated, the proportion of the nitre being one-half to 5% with respect to the weight of the article or articles being treated.

5. A bath for treating puered skins or hides for preserving them and to increase the uniformity and refine the grain thereof

comprising water, alum, salt, nitre and formaldehyde substantially in the proportions as set forth.

In testimony whereof, I affix my signature hereto.

HARRY DODGE.